

April 30, 1929.

E. GATHMANN

1,711,052

METHOD OF PRODUCING STEEL INGOTS

Filed June 22, 1928.

2 Sheets-Sheet 1



INVENTOR  
*Emil Gathmann.*

BY *Baldwin & Hight*  
ATTORNEYS

April 30, 1929.

E. GATHMANN

1,711,052

METHOD OF PRODUCING STEEL INGOTS

Filed June 22, 1928

2 Sheets-Sheet 2

PLATE



INVENTOR

*Emil Gathmann*  
BY *Baldwin & Wright*

ATTORNEYS

PLATE

## UNITED STATES PATENT OFFICE.

EMIL GATHMANN, OF BALTIMORE, MARYLAND.

## METHOD OF PRODUCING STEEL INGOTS.

Application filed June 22, 1928. Serial No. 287,557.

My invention relates primarily to the method of producing steel or alloy ingots which shrink or contract in passing from the liquid to the solid state and which are subsequently rolled, pressed or otherwise worked into commercial shapes or forgings.

In speaking of an ingot it is to be understood that I refer to one cast in a suitably proportioned big-end-up tapered mold, such as is described in Patents No. 1,049,573 of January 7, 1913 and No. 1,643,241 of September 20, 1927 granted to me.

A fundamental requirement in the production of a physically sound and relatively homogeneous steel ingot is that of suitable deoxidation of the bath after proper chemical analysis has been obtained. In addition to this, the metal must be properly finished in the ladle prior to teeming it into the mold.

When teemed at suitable temperature into an iron mold having relatively heavy chamber walls, metal so finished will solidify in several distinct phases, the initial solidification being due to contact of the molten metal with

the walls defining the mold chamber. This solidification is practically coincident with the entrance of the steel into the mold and is only of skin thickness. The greater mass of the ingot then solidifies within this initially-

formed skin by crystallization of a dendritic form, which starts at right angles to the skin surface and progresses from the sides and bottom to the center of the ingot. The rate of solidification decreases as the ingot skin

increases in thickness and the matrix walls of the mold become heated, at which time solidification proceeds not only by the formation of dendritic crystals, but also by the formation of equiaxial or free crystallization. The

more rapid the solidification of the body of the ingot, the greater will be the number of independent nuclei from which solidification proceeds. As a result of such rapid solidification, the formation of the dendritic crystals,

which proceeds inwardly and at right angles to the initial skin of the ingot, prevents or at least greatly reduces so-called clotted segregation. What may be termed a land-locking type of solidification occurs due to the growth

of the dendrites retarding free emigration or segregation of nonmetallic impurities, or matter not in solid solution in the molten steel.

It is now well-known to those familiar with the art that thoroughly deoxidized steel is of greater volume when molten than the same

weight of metal when solidified, this reduction in volume or "shrinkage" having been ascertained to be somewhere between 3% and 5% in ordinary carbon steels, the exact amount of shrinkage depending primarily upon the pouring temperature. The method

of solidification, or the extent of growth of dendritic and equiaxial crystals, determines the position and type of the shrinkage cavity formed in the ingot during the process of solidification. By keeping a continuous supply of molten metal above the solidifying crystals it is theoretically possible to produce an ingot without any shrinkage cavity at all, the shrinkage in volume of the metal resulting only in a shortening of the ingot.

The primary object of my invention is to so shape and solidify steel ingots that a greater yield of physically sound, substantially homogeneous material is obtainable from the solidified ingot than has heretofore been considered possible in tonnage practice.

A further object of my invention is to so cool and solidify the molten mass of the ingot from the bottom progressively upwardly that molten metal is continuously superimposed upon the crystallizing portion of the ingot, until finally the uppermost part of the metal, or that contained within the top zone of a suitably constructed shrink head casing, has cooled or frozen. In other words, I abstract the heat of the ingot first at the bottom and thence progressively upward, causing the isotherms or lines of abstraction of heat to be swung downwardly from the usual nearly vertical lines to lines progressively flattening out from bottom to top of the ingot structure. Since the isothermal lines at the top of the ingot are nearly horizontal, I obtain a flatter and a shallower shrinkage cavity, all of which is contained in the uppermost portion of the ingot, so that only 10% or even less of the total volume of the molten ingot metal need be contained within the hot top in order to assure of physical soundness in the ingot body.

The method covered by U. S. Patent No. 1,049,573, issued to me January 7, 1913, provides for the rapid cooling of approximately 85% of the mass of molten metal from the bottom towards the top and the retarding of the cooling and solidification of approximately 15% at the top. Many million tons of ingots have since been produced by this method, an average yield of from 80% to 82% of sound, finished product being obtained

from each ingot. My present invention, however, as before stated, provides means for relatively rapid cooling of from 90% to 92% of the mass of molten steel, whereby I obtain 5 a greater yield, approximately 88% to 90% of sound, substantially homogeneous product from the solidified ingot.

The accompanying drawings illustrate a type of mold and hot top for carrying out my 10 invention. It is to be understood, however, that molds and hot tops of other contours, either in vertical or horizontal cross section, may be employed within the limits herein-after specified, without departing from the 15 scope of my invention.

Figure 1 shows a vertical central section of an ingot mold and the molten metal of an ingot immediately after being cast therein.

Figure 2 shows a vertical section of an ingot 20 mold containing an ingot which has solidified therein.

Figure 3 is a sectional view through line 3—3 of Figure 4.

Figure 4 is a sectional view on line 4—4 of 25 Figure 3.

In carrying out my invention it is essential that the metallic mold employed is so constructed that the heat of the ingot metal cast therein will be extracted and the ingot solidified along isothermal lines 1, which progressively flatten out from the bottom to the top of the ingot structure as the solidification of the molten metal proceeds progressively from 30 bottom to top.

35 The chamber of the metallic mold 2 forming or defining the body of the ingot 3 has relatively heavy bottom and side walls 4, the combined cross-sectional area of which is approximately twice that of the horizontal sectional area of the mold chamber at the lower portion 5 and about of approximately equal area to that of the mold chamber at the upper portion 6. In other words, the chill walls of the mold chamber become thinner and less 40 heat absorptive from the bottom towards the top. The preferred relative dimensions of the ingot mold chamber are indicated in my patent of September 20, 1927, referred to above.

50 Mounted upon the upper face of the metallic, heat-absorbing mold body 2 is a hot top or shrink head casing of the type described in my U. S. Patent No. 1,696,395 of December 25, 1928. The shrink head casing as a whole 55 in its preferred form is designated by 7 and is constructed primarily of a highly refractory fire clay 8, the sintering point of which is preferably somewhat higher than the pouring temperature of liquid steel. The core

60 portion 9 of the hot top or shrink head casing walls is of an exceedingly porous nature, being permeated with microscopic cells. For this core portion I preferably employ infusorial earth and a binder, which allows but 65 little absorption and practically no conduc-

tion of heat through the walls of the casing. The exterior walls 8, however, are made homogeneous, dense and highly refractory to the heat of the molten ingot metal. The casing 7, as described, can be formed in various 70 ways, details of several methods of manufacture being described in the aforesigned co-pending application.

In carrying out my present method of ingot production, I have found it essential, in order 75 to obtain the best results, to not only conserve the heat at the vertical portions of the shrink head of the ingot, but also at the upper face thereof, substantially as described in my Patent No. 1,049,573 of January 7, 1913. For 80 this purpose I employ a material 10 that is neutral when in contact with the molten steel and the particles of which material contain microscopic cells so that the escape of heat from the top of the ingot is prevented. I have 85 found that complete insulation may be obtained with as little as an inch thickness of such material, powdered infusorial earth, diatomite or the like, indicated at 10 in Figures 1 and 2 of the drawings being preferred. 90

By the use of a mold and shrink head casing of the type described, I prevent radiation of heat from the upper sides and top portion of the ingot and I am enabled to materially 95 reduce the volume of the chamber of the shrink head casing. I have found from experiments that the percentage of steel in the heat-conserving mold top or shrink head casing may be reduced to as little as 8% to 10% of the entire volume of the molten ingot. The 100 yield of sound steel in the body of the ingot is thus increased some 11% to 13% above that previously considered possible in the commercial production of mill ingots, effecting a 105 saving of \$2.50 to \$3.00 a ton in the ordinary grades of carbon forging steel.

It is thus apparent that in practicing my method of ingot production, wherein the proportion of rapid cooling and solidification extend to at least 90% of the vertical mass of 110 the ingot and wherein a reservoir of molten steel, amounting to 10% or less, is superimposed upon the solidifying crystals in the body of the ingot until the entire ingot and sink head have become cooled and solidified 115 from the bottom upwardly. I obtain a steel that is superior in its response to forging and heat treatment and the finished product of which is of a higher quality than that produced from ingots made by methods heretofore known to the art, at the same time effecting a saving by increasing the yield of sound product obtainable from the ingot.

I claim as my invention:

The herein described method of producing 125 sound steel ingots by which the defective portion of the ingot is reduced, which consists in deoxidizing the molten metal in the bath after the desired chemical analysis is obtained, transferring the metal to a pouring 130

ladle and subjecting it to further deoxidizing or finishing treatment, then teeming the metal into a mold for the formation of an ingot, progressively accelerating by absorption the 5 radiation of heat from the forming ingot from the bottom thereof towards the top for approximately 90% of the mass of molten metal and in substantially suspending the absorption of heat from the ingot at the upper 10 portion thereof and positively retarding the radiation of heat therefrom for approximately 5% to 10% of the upper por-

tion of said forming ingot, to thus cause the upper portion of the mass to feed deoxidized molten metal to the forming ingot to compensate for the shrinkage in the body of the ingot while the metal is cooling and solidifying, and to thus cause the physically defective or porous portion of the ingot to be entirely confined within the upper 5% to 10% therefor. 15 20

In testimony whereof, I have hereunto subscribed my name.

EMIL GATHMANN.